

# United States Patent Office

2,898,297

Patented Aug. 4, 1959

1

2,898,297

## GREASE COMPOSITION AND METHOD OF PREPARATION THEREOF

John E. Schott, New York, N.Y., assignor to Socony Mobil Oil Company, Inc., a corporation of New York

No Drawing. Application December 29, 1958  
Serial No. 783,158

19 Claims. (Cl. 252—36)

This invention has to do with new grease compositions, particularly grease compositions characterized by a number of desirable properties. The novel greases contain soaps of coconut oil balanced with soaps of intermediate and high molecular weight fatty acids and salts of low molecular weight fatty acids, together with additional ingredients.

This application is a continuation-in-part of my application Serial No. 524,296, filed July 25, 1955, now abandoned.

It is well known that greases lose some or all of their effectiveness when subjected to severe operating conditions, and particularly when subjected to high temperature operations. In lubricating machine parts, for example, it is essential that a grease retain its useful form; failure to do so results in a high consumption of the grease and frequent servicing. In general, available greases suffer from a marked tendency to change in character when used over a wide range of temperature, notably at high temperatures of the order of 250–350° F. and higher. Some conventional greases are characterized by excessive softening when exposed to such high temperature operations, thereby being expelled too rapidly from the area being lubricated to provide efficient lubrication.

The action of water—whether salt or fresh water—may cause the grease to thin out into a liquid which leaks out from the lubricated surfaces. This is a prime consideration inasmuch as grease-lubricated machine parts are encountered in port installations, on deck of navy and marine vessels, in steel rolling mills, in water pumps of all kinds, in mining machinery, in oil-well drilling equipment, etc. In many of such instances, relatively high operating temperatures develop, such that even lime base greases, which are highly resistant to water, become unstable. While a number of modifying agents have been incorporated in various grease types to improve their stability, such modifying agents have generally been relatively expensive and some have depreciated one or more other desirable characteristics of the grease.

On the other hand, many of the past and present day greases have failed to provide resistance to corrosion in humid air of the machine parts which the greases should protect. Such greases have generally been hygroscopic in character and, as a result, harden appreciably. In this respect, they have proven inadequate.

Present day demands for greases have also given rise to the need for greases characterized by excellent extreme pressure character, oxidation stability and long bearing performance life. While some success has been realized in providing greases with extreme pressure characteristics, for example, the greases so characterized have fallen far short of having satisfactory oxidation stability or good bearing performance. Correspondingly there has been success in the development of greases having a high degree of oxidation stability; but, here again, the same grease will generally have an undesirably low extreme pressure value.

2

It has now been found that a grease characterized by all of the foregoing desirable properties can be prepared from certain soaps and salts of the following acids, interrelated as shown below:

|    | Acid                       | No. of Carbon Atoms | Wt. Percent of Total Acid |
|----|----------------------------|---------------------|---------------------------|
| 10 | Low Molecular Weight       | 1-6                 | 10-50                     |
|    | Intermediate Molecular Wt. | 7-12                | 5-50                      |
|    | High Molecular Weight      | 13-22 or more       | 5-40                      |
|    | Coconut Oil Acids          | 6-18                | 25-60                     |

It is to be understood that the coconut oil acids generally constitute about 86 to about 89% by weight of coconut oil.

The foregoing percentage ranges are applicable broadly to the grease compositions of this invention. With blends of oils having a viscosity of about 70 seconds (S.U.V.) at 210° F., and a V.I. between 0 and 60, the optimum percentage range is the following:

| Acid:                         | Wt. percent of total acid |
|-------------------------------|---------------------------|
| Low molecular weight          | 28                        |
| Intermediate molecular weight | 17                        |
| High molecular weight         | 14                        |
| Coconut oil acids             | 41                        |

That this relationship is critical is revealed by the fact that when an insufficient quantity of a low molecular weight acid, such as acetic acid, is used, the grease made therewith is semi-fluid and has an undesirably low dropping point. Correspondingly, an excessive amount of an acid such as acetic produces a soap structure which is difficult, if not impossible, to disperse in a stable state in the oil vehicle. A similar influence is seen in the use of too little, or an excess of an intermediate molecular weight acid, such as caprylic. An insufficient quantity of caprylic acid generally causes the product to harden excessively in storage; and an excess of caprylic acid causes the product to bleed excessively in storage. An improper balance is realized, too, when an insufficiency or excess of high molecular weight acid, such as stearic is used. Too little stearic acid results in a product of excessive fluidity in oil-bleeding in storage and poor worked stability; and an excess of stearic acid is responsible for undesirable changes in storage, lowered dropping point, and poor response to water contamination.

Typical of the low molecular weight acids contemplated herein are: acetic, propionic, butyric, valeric, and caproic. Of these, acetic is particularly desirable because it provides outstanding products.

Typical of intermediate molecular weight acids are: heptanoic, caprylic, pelargonic, capric, lauric; mono hydroxy substituted acids such as alpha-hydroxy decanoic, mixed unsubstituted C<sub>8</sub>, C<sub>10</sub>, C<sub>12</sub>, having a methyl side chain, such acids being obtained by the Oxo process. Caprylic, capric and pelargonic are particularly advantageous of such acids.

Illustrative of the high molecular weight monocarboxylic acids of the invention are: saturated aliphatic acids such as myristic, palmitic, stearic, etc.; mono unsaturated aliphatic acids such as oleic; mono hydroxy substituted acids such as 12-hydroxy stearic acid. Preferred are the unsubstituted saturated acids, particularly stearic and palmitic acids.

It is to be understood, of course, that more than one acid of a given type can be used so long as the balance recited above is maintained.

As indicated above, another component of the greases of this invention going to make up the desired soaps, is coconut oil. This oil contains glycerides, a large proportion of the fatty acids of which have from about

12 to about 14 carbon atoms per molecule. As is well known in the art, however, coconut oil also contains other glycerides the acids of which have as few as about 6-10 carbon atoms per molecule and other acids which have as many as about 18 carbon atoms per molecule. In addition to the said acids, there is the equivalent of about 11 to about 14% by weight of glycerine in coconut oil. A typical coconut oil used herein has the following characteristics:

|                       |                |
|-----------------------|----------------|
| Saponification value  | 260            |
| Iodine No.            | 10             |
| Titer, ° C.           | 23             |
| Composition of acids: | Percent by wt. |
| Caprioc               | 0.5            |
| Caprylic              | 8.5            |
| Capric                | 7.5            |
| Lauric                | 47.5           |
| Myristic              | 18.5           |
| Palmitic              | 7.5            |
| Stearic               | 2.5            |
| Oleic                 | 5.0            |
| Linoleic              | 2.5            |
| Total                 | 100.0          |

As shown hereinafter, greases of superior quality are obtained when either coconut oil or comparable quantities of glycerine and coconut oil fatty acids, are used. However, greases formed from coconut oil according to this invention, are exceptional with respect to oxidation stability and, for this reason, coconut oil is particularly preferred.

In addition to coconut oil, and its saponification products coconut oil fatty acids and glycerine, other nut or kernel oils in which the fatty acids are predominantly in the C<sub>12</sub>-C<sub>14</sub> range are considered suitable for use in preparing the greases of this invention. Typical of such oils are palm kernel oil and babassu kernel oil. The distribution of acids present in such oils is given below, weight percent being shown:

|          | Palm Kernel Oil Acids | Babassu Kernel Oil Acids |
|----------|-----------------------|--------------------------|
| Caproic  | 2.7-3.0               | Trace                    |
| Caprylic | 3.0-7.0               | 6.5                      |
| Capric   | 47.0-52.0             | 2.7                      |
| Lauric   | 14.1-15.0             | 45.8                     |
| Myristic | 7.5-8.8               | 19.9                     |
| Palmitic | 1.3-2.5               | 6.9                      |
| Stearic  | 16.0-18.5             | 18.1                     |
| Oleic    | 0.7-1.0               |                          |
| Linoleic |                       |                          |

Palm kernel and babassu kernel oils contain approximately the same percent by weight of glycerine as coconut oil. The kernel oils can be used in place of or together with coconut oil. Here too, it is contemplated that the kernel oils be used or that comparable quantities of glycerine and the kernel fatty acids be used.

The metal component of the salts and soaps formed from the foregoing acids, in the preparation of the greases of this invention, is primarily calcium. However, as much as about 10 to about 15%—on a chemical equivalent basis—of the calcium used may be replaced by barium such that the finished grease will contain a mixture of calcium and barium soaps. The corresponding metal oxides, metal hydroxides and metal carbonates can be reacted with the aforesaid acids in order to provide the desired salts and soaps.

In addition to the salts and soaps described above, the greases contemplated herein contain a lead compound. A lead compound or compounds are formed in situ by means of reaction between the said acids and lead-containing charge material or reactant such as lead acetate and litharge (PbO), particularly the latter. How-

ever, it is also contemplated herein, that a lead compound of any one or more of the acids of the character recited above can be incorporated into the grease rather than being formed in situ.

Another component of the greases of this invention is a chlorine-containing, sulfur-containing, chlorine-and-sulfur-containing, phosphorus-containing, phosphorus-and-chlorine-containing, phosphorus-and-sulfur-containing, or phosphorus-and-sulfur-and-chlorine-containing organic compound known in the art as an extreme pressure agent. Among such compounds are the following, which are particularly effective and as such are preferred:

15 Methyl dichlorostearate  
Chlorinated sperm oil one example of which is "Alpha-Chlor 33"

Sulfurized sperm oil

Sulfurized lard oil

20 Aryl, alkyl and alkyl-aryl phosphates typical of which is tricresyl phosphate

"Alpha-Chlor 33" is a chlorinated sperm oil. It is sold by the Carlisle Chemical Works under the trade name "Alpha-Chlor 33" and is described by its properties in the following manner:

Chlorine, percent by weight 33.

Lbs./gal. at 60° F. 9.6.

Pour point, ° F. 5.

30 Flash point None.

Viscosity, @ 210° F., SSU 200.

Solubility Completely soluble in most petroleum oils, partially soluble in solvent refined oils.

The mineral oil component of the greases of this invention can vary considerably in character. In general, such oils are characterized by a viscosity (S.U.V.) greater than about 40 seconds at 100° F., preferably from about 60 to about 6,000 seconds at 100° F. It has been found, however, that the character of mineral oil used materially influences the character of the grease composition. A blend of a solvent-refined naphthenic oil having a viscosity of 500 seconds at 100° F., and a viscosity index of 60, when blended with a naphthenic bright stock having a viscosity of 130-140 seconds at 210° F., such that the final blend has a viscosity at 210° F. of about 70, has proven to be particularly desirable.

45 In place of all or part of the mineral oil component, other oils of lubricating viscosity can also be used, such oils including synthetic vehicles comprising esters of dibasic acids. Typical of such synthetic oils are: di-(2-ethyl hexyl) sebacate, dibutyl phthalate, di-(2-ethyl hexyl) adipate. Other suitable synthetic oils are esters of poly alcohols and monocarboxylic acids, such as polyethylene glycol di-(2-ethyl hexoate).

50 The oil component or vehicle, and the components mentioned herein above, are used in the grease compositions in the proportions (percent by weight of the finished grease composition) as indicated in the following tabulation:

| Component                                                                | Range | Preferred Range |
|--------------------------------------------------------------------------|-------|-----------------|
| Oil vehicle                                                              | 50-98 | 70-90           |
| Calcium or Calcium-barium salts and soaps of coconut oil and other acids | 1-40  | 5-25            |
| Lead compound expressed as PbO                                           | 0.5-5 | 1-2             |
| Extreme pressure agent                                                   | 1-10  | 2               |
| Oxidation inhibitor                                                      | 0-1   | 0.2-0           |

65 It has been found that greases of outstanding character are realized when a novel technique or procedure is followed. It appears that the order of these steps is critical in nature, since departure from the said order results in a less advantageous product. By way of illus-

tration, a batch of grease is formed in the manner described in Example 1 below.

#### EXAMPLE 1

A Stratco contactor is preheated to about 250° F. and is then charged in the order indicated with oil, alkali and acids:

|                                                                                     |                |
|-------------------------------------------------------------------------------------|----------------|
| Mineral oil solvent refined naphthenic oil,<br>60 V.I., 500 sec., S.U.S. at 100° F. | 56 lbs.        |
| Lime flour                                                                          | 9 lbs. 7 oz.   |
| Acetic acid                                                                         | 8 lbs. 5 oz.   |
| Water                                                                               | 4 lbs.         |
| Caprylic acid                                                                       | 5 lbs.         |
| Coconut oil                                                                         | 12 lbs. 11 oz. |
| Hydrogenated tallow fatty acids                                                     | 4 lbs. 3 oz.   |
| Litharge                                                                            | 3 lbs.         |

The agitator of the Stratco contactor is in motion at all times during the addition of the aforesaid materials. The contents of the contactor are heated to about 345° F. by means of the hot oil circulating system forming a part of the Stratco contactor. Approximately one hour is required to heat the contents from the initial temperature of 250° F. to about 345° F. The pressure within the contactor reaches a value of about 100 lbs./sq. in. under such conditions. Heat is discontinued and the contents are transferred (blown over) into a preheated steam kettle which is of the open paddle kettle type.

The course of reaction is determined by withdrawing a sample of the soap from the contactor. In a typical preparation, the alkalinity of the contents, determined as percent by weight CaO, is between about 0.5 and about 0.7%. (Determined in accordance with ASTM Method D128-47, modified by using a 50-50 mixture of water and alcohol.) When the alkalinity value is within this range the contents are dehydrated.

When the materials from the contactor are transferred to the open paddle kettle, the temperature thereof drops to about 300° F. as a result of moisture loss and as a result of the influence of atmospheric temperature. The materials now in the open kettle are heated and paddled for about 1½ hours at 300 to 320° F. Thereupon, 44 lbs. of the oil described above and 30 lbs. of a naphthenic bright stock having a viscosity of 130-140 seconds (S.U.S.) at 210° F. and a V.I. of less than 0, are added. Heating of the open kettle is discontinued and the contents thereof are recycled through a high pressure homogenizer as described in Armstrong Patent 2,704,363, at about 3,000 lbs. per sq. in. until the temperature drops to about 180° F. When the temperature is about 190° F., a quantity (5 lbs. 3 oz.) of "Alpha-Chlor 33" is added. The worked penetration is adjusted to about 290-300 by adding a mineral oil blend to the product. The mineral oil blend comprises an 80-20 mixture of the initial oil and of the naphthenic bright stock, respectively, described above. This will generally call for from 0 to about 20 lbs. of oil blend in order that the penetration value be realized. The product is then filled in packages through the homogenizer at 3,000 lbs. per sq. in. at 180° F.

Typical results of pilot plant batches, such as the batch described hereinbefore, are given below in the following tabulation:

|                                                                                    |                                              |
|------------------------------------------------------------------------------------|----------------------------------------------|
| Timken OK load in lbs.                                                             | 45.                                          |
| Color                                                                              | Brown.                                       |
| ASTM Motormatic worker test<br>after 100,000 strokes with $\frac{1}{4}$ "<br>holes | 312-330.                                     |
| Oxidation stability, lb. drop in<br>hours, ASTM Bomb at 210° F.                    | 10#/200 hrs. with no<br>oxidation inhibitor. |
| Oxidation stability, lb. drop in<br>hours, ASTM Bomb at 210° F.                    | 4#/500 hrs. with 0.5%<br>Ionol.              |
| Penetration                                                                        | 290/300.                                     |

|                                                                       |                                             |
|-----------------------------------------------------------------------|---------------------------------------------|
| Separability in percent, 100 hrs.,<br>7.5#/sq. in. pressure at 77° F. | 4.9.                                        |
| Bleeding, in percent, 50 hrs. at<br>210° F., MIL-G-3278               | 3.5.                                        |
| Dropping point, ° F.                                                  | 500 plus.                                   |
| Salt spray, MIL-G-10924                                               | 100 hours plus.                             |
| Performance life in loaded Navy<br>tester at 257° F.                  | 1500 hrs. without oxida-<br>tion inhibitor. |

|                                                         |                               |
|---------------------------------------------------------|-------------------------------|
| 10 Performance life in loaded Navy<br>tester at 257° F. | 3500 hrs. with 0.5%<br>Ionol. |
| Apparent viscosity at 30° F.                            | 860.                          |

|    |                                                                                                                                                                                                                                                                                                                                                                                                                                                                                                                             |
|----|-----------------------------------------------------------------------------------------------------------------------------------------------------------------------------------------------------------------------------------------------------------------------------------------------------------------------------------------------------------------------------------------------------------------------------------------------------------------------------------------------------------------------------|
| 15 | Several unusual features are shown in the aforesaid tabulation of data. It is to be noted that an extreme pressure value as high as 45 pounds, together with excellent oxidation stability and long bearing performance life, is a relationship not hitherto realized in the preparation of greases. High extreme pressure values have been obtained in the past but a grease so characterized has not had satisfactory oxidation stability or bearing performance life at elevated temperatures such as 200° F. and above. |
| 20 | Similarly, excellent oxidation stability or bearing performance life have been realized yet the extreme pressure value has been lacking or so low as to be negligible. Here, for the first time, all three features are together in excellent balance.                                                                                                                                                                                                                                                                      |
| 25 | Results obtained with other typical greases of this invention are shown in Table I below. In the greases shown here, extreme pressure agents other than "Alpha-Chlor 33" were used in the grease, containing the latter, defined hereinabove.                                                                                                                                                                                                                                                                               |

|    |                                                                                                                                                                                                                                               |
|----|-----------------------------------------------------------------------------------------------------------------------------------------------------------------------------------------------------------------------------------------------|
| 30 | Results obtained with other typical greases of this invention are shown in Table I below. In the greases shown here, extreme pressure agents other than "Alpha-Chlor 33" were used in the grease, containing the latter, defined hereinabove. |
|----|-----------------------------------------------------------------------------------------------------------------------------------------------------------------------------------------------------------------------------------------------|

Table I

| Extreme Pressure Agent, Percent<br>by Wt. | Timken<br>OK<br>Load,<br>Lbs. | ASTM<br>Penetra-<br>tions | Motormatic<br>Worker Test,<br>5,000×Penetra-<br>tion |
|-------------------------------------------|-------------------------------|---------------------------|------------------------------------------------------|
| Methyl dichlorostearate, 2.6.....         | 35                            | 208/212                   | 255                                                  |
| Methyl dichlorostearate, 5.2.....         | 40                            | 235/238                   | 346                                                  |
| Sulfurized lard oil, 5.0.....             | 45                            | 224/244                   | 277                                                  |
| Tricresyl phosphate, 2.6.....             | 40                            | 207/226                   | 289                                                  |

45 The nature of present invention is illustrated further by the following examples, wherein products were formed with either barium or sodium substituted for calcium in the grease described by Example 1. Comparison is then set out in Table II of the calcium grease and the products formed with barium and with sodium.

|    |                                                                      |
|----|----------------------------------------------------------------------|
| 55 | The materials used are the following:                                |
|    | Mineral oil, solvent refined, 500 S.U.S.<br>@ 100° F..... 20 pounds. |
|    | Barium hydroxide octahydrate..... 20 pounds.                         |
| 60 | Acetic acid..... 4 pounds 2½ oz.                                     |
|    | Caprylic acid..... 2 pounds 8 oz.                                    |
|    | Coconut oil..... 6 pounds.                                           |
|    | Hydrogenated tallow fatty acids..... 2 pounds 1½ oz.                 |
|    | Litharge..... 1 pound 8 oz.                                          |

65 The Stratco contactor was preheated to 220° F. and the aforementioned materials were charged thereto. The charge was heated to 345° F. During a period of 1 hour and 10 minutes, a pressure of 105 pounds per square inch developed. The contents of the contactor were then blown over into a 100 pound drum. The product was semi-fluid. The product was then transferred to a hot steam kettle and was heated and paddled therein at or slightly above 300° F. The product remained semi-fluid. While at a temperature of 300° F., it was then homogenized through a Manton Gaulin unit, at

about 3000 p.s.i., and cooled to 180° F. Since no grease-like material developed, additional oil was not added. The product when cooled and homogenized had a semi-fluid consistency.

## EXAMPLE 3

The Stratco contactor was preheated to 220° F. and the following materials were charged thereto in the order in which they are listed below:

|                                                                                 |                  |
|---------------------------------------------------------------------------------|------------------|
| Mineral oil, solvent, refined, naphthenic, 60 V.I., 500 secs. S.U.S. at 100° F. | 56 pounds.       |
| Sodium hydroxide                                                                | 10 pounds.       |
| Acetic acid                                                                     | 8 pounds 5 oz.   |
| Water                                                                           | 4 pounds.        |
| Caprylic acid                                                                   | 5 pounds.        |
| Coconut oil                                                                     | 12 pounds 11 oz. |
| Hydrogenated tallow fatty acids                                                 | 4 pounds 3 oz.   |
| Litharge                                                                        | 3 pounds.        |

As in Example 2, the charge was heated to 345° F. One hour and 15 minutes were required to heat the charge from 220° F. to 345° F. A pressure of 100 p.s.i. developed in the contactor. The reaction mixture was blown over into a 120 pound drum, and was then transferred to a hot steam kettle. The mixture from the Stratco was soft and mushy. The alkalinity was determined to be 0.90 percent by weight of sodium hydroxide; this was determined by ASTM Method D128-47, modified as indicated above.

The reaction mixture was heated in the steam kettle for 1½ hours, when a temperature of 320° F. was reached. Heating of the kettle was continued for 1½ hours. Fifty pounds of grease was removed from the kettle. Twenty-two pounds of the same oil as used in the charge, was added to the balance of the reaction mixture remaining in the steam kettle. Heating of the steam kettle was discontinued. The contents of the steam kettle were then homogenized at 3000 p.s.i. in a Manton Gaulin unit. The homogenized product was cooled from 320° F. to 180° F. during a 1½ hour period. "Alpha-Chlor 33," 2 pounds and 6 ounces, were then added to the cooled product. The unworked and worked penetrations of the product were in excess of 420.

Comparison of the products formed in Examples 1, 2 and 3 are shown in Table II, following.

Table II

| Example No.                                 | 1       | 2          | 3          |
|---------------------------------------------|---------|------------|------------|
| Type of Soap                                | Calcium | Barium     | Sodium     |
| Acetic Acid, wt. percent                    | 4.67    | 4.67       | 4.67       |
| Caprylic Acid, wt. percent                  | 2.81    | 2.81       | 2.81       |
| Coconut Oil, wt. percent                    | 7.14    | 7.14       | 7.14       |
| Hydrogenated Tallow Fatty Acid, wt. percent | 2.36    | 2.36       | 2.36       |
| Litharge, wt. percent                       | 1.69    | 1.69       | 1.69       |
| Mineral Oil                                 | Balance | Balance    | Balance    |
| Metal Component                             | Calcium | Barium     | Sodium     |
| Calcium Ion Equivalent <sup>1</sup>         | 2.05    | 2.95       | 2.95       |
| Type of Product                             | Buttery | Semi-Fluid | Semi-Fluid |
| Penetration, Unworked/Worked                | 290/300 | 420+/420+  | 420+/420+  |

<sup>1</sup> 2.95 equals 5.47 weight percent of Ca(OH)<sub>2</sub>

$$\frac{40}{74} \times 5.47 = 2.95$$

As shown by Examples 1 through 3 calcium is useful in forming excellent greases of the character contemplated herein, whereas barium and sodium can not be used in place of calcium. Although a complete substitution can not be made, a minor proportion of calcium can be replaced by barium. This is demonstrated by Example 4 following.

## EXAMPLE 4

A grease was formed from the following materials:

|                                         | Wt. percent |
|-----------------------------------------|-------------|
| 5. Mineral oil, identified in Example 1 | 56.75       |
| Naphthenic bright stock in Example 1    | 18.70       |
| Lime                                    | 4.45        |
| Barium hydroxide                        | 0.50        |
| Litharge                                | 1.50        |
| 10 Acetic acid                          | 4.16        |
| Caprylic acid                           | 2.5         |
| Coconut oil                             | 6.34        |
| Hydrogenated tallow fatty acids         | 2.5         |
| 15 Alpha-Chlor 33                       | 2.6         |

The procedure used in preparing this grease involved charging a Stratco contactor with the components listed, except for the naphthenic bright stock and Alpha-Chlor 33 and one-half of the mineral oil. The charge was heated and maintained at 320-330° F. for two hours at a pressure of 40-45 p.s.i. Pressure was then reduced to atmospheric. The charge was heated at 320-330° F. for an additional 2 hours, during which time the remaining one-half of the mineral oil was added thereto. 20 Heating of the contactor was discontinued. The naphthenic bright stock was added. The resulting mixture was cooled to 170° F. Alpha-Chlor 33 was added. The product was then homogenized thru a Charlotte mill, having a clearance of 0.002 inch. The product had an alkalinity of 0.27% CaO (determined as identified above). The grease so formed had the following characteristics:

|                                                           |         |
|-----------------------------------------------------------|---------|
| Penetration, worked/unworked                              | 294/312 |
| 35 ASTM Motormatic worker test after 5000 strokes with ¼" | 354     |

As revealed by the foregoing properties, a satisfactory grease is formed by replacing some of the calcium component with barium. However, when as much as twenty 40 percent (chemical equivalent basis) of the lime used was substituted by barium hydroxide octahydrate, a semi-fluid product was obtained.

Comparison has also been made of the calcium grease described in Example 1, above, in which coconut oil was used, with a grease prepared with comparable quantities of glycerine and coconut oil fatty acids. The latter grease is described in Example 5 below.

## EXAMPLE 5

50 The following charge was added to a Stratco contractor, which had been preheated to 250° F.:

|                                                                      |                 |
|----------------------------------------------------------------------|-----------------|
| Mineral oil, solvent refined naphthenic, 500 secs. S.U.S. at 100° F. | 56 pounds.      |
| 55 Lime flour                                                        | 9 pounds 1 oz.  |
| Acetic acid                                                          | 8 pounds 5 oz.  |
| Water                                                                | 4 pounds.       |
| Caprylic acid                                                        | 5 pounds.       |
| Coconut oil fatty acids                                              | 11 pounds 4 oz. |
| 60 Hydrogenated tallow fatty acids                                   | 4 pounds 3 oz.  |
| Litharge                                                             | 3 pounds.       |
| Glycerine                                                            | 1 pounds 8 oz.  |

The charge materials were heated to 345° F. during a period of 1¼ hours. A pressure of 105 p.s.i. was developed in the contactor. The reaction mixture was blown over into a 100 pound drum and was then transferred to a hot steam kettle. The mixture was firm. After the mixture had been paddled in the kettle for 15 minutes, a sample was taken for an alkalinity determination; the mixture had an alkalinity of 0.15% CaO (alkalinity determined as indicated above). Half of the mixture was removed from the kettle.

The mixture remaining in the kettle was then heated 75 to 320° F. during a 1½ hour period. Additional mineral

oil (the same as charged), 22 pounds, was added to the mixture. Then, 15 pounds of another mineral oil was added; this was a naphthenic bright stock having a viscosity of 130-140 seconds (S.U.S.) at 210° F. Heating of the kettle was discontinued. The resulting mixture was paddled and then was passed through a Manton Gaulin unit (operating at 3000 p.s.i.) from 320° F. to 180° F. over a 1½ hour period. At this stage, 2 pounds and 10 ounces of "Alpha-Chlor 33" was added. The mixture so formed was paddled for a ¼ hour, and 10 pounds of an oil blend was added. The oil blend comprised the solvent refined oil and the naphthenic bright stock identified above. The resulting product was paddled for ¼ hour. A 10 pound sample was taken at this stage; it was identified as sample 1. To the remainder of the product was added 0.5 percent by weight of Ionol (2-6-ditertiary-butyl-4-methylphenol). The resulting product was paddled for ¼ hour and a sample (sample 2) was drawn out through the Manton Gaulin unit.

Data for the products of Examples 1 and 5 are shown in Table III following.

Table III

| Example No.                                                  | 1            | 5            |
|--------------------------------------------------------------|--------------|--------------|
| Coconut Oil                                                  | Yes          |              |
| Coconut Oil Fatty Acids                                      |              | Yes          |
| Glycerine                                                    |              | Yes          |
| Properties:                                                  |              |              |
| Penetration, Worked                                          | 300          | 288          |
| Timken OK Load, lbs.                                         | 45           | 45           |
| Oxidation Stability, lb. drop in hours, ASTM Bomb @ 210° F.— | 10#/200 hrs. | 10#/126 hrs. |
| no oxidation inhibitor                                       | 4#/500 hrs.  | 10#/286 hrs. |
| with 0.5% oxidation inhibitor <sup>1</sup>                   |              |              |

<sup>1</sup> Ionol.

Attention is drawn to the oxidation stability values set out in Table III. Surprisingly, the grease of Example 1 is superior to that of Example 5. For some reason, coconut oil appears to cooperate with the other materials used in the preparation to provide a product of superior oxidation stability; whereas, glycerine and coconut oil fatty acids cooperate to a substantially lesser extent.

Further illustration of the unusual compositions of this invention is provided by Example 6. In this example, composition 6(c) is compared with composition 6(a) and 6(b).

#### EXAMPLE 6

(a) A grease was prepared by the procedure given in Example 1, from the following materials:

| Percent by weight                    |       |
|--------------------------------------|-------|
| Mineral oil <sup>1</sup>             | 58.23 |
| Naphthenic bright stock <sup>1</sup> | 19.20 |
| Lime flour                           | 4.87  |
| Acetic acid                          | 4.16  |
| Caprylic acid                        | 2.50  |
| Coconut oil                          | 6.34  |
| Hydrogenated tallow fatty acids      | 2.10  |
| Alpha-Chlor 33                       | 2.60  |

<sup>1</sup> Same as described in Example 1, above.

(b) A grease differing principally from that described as 6(a) in the incorporation of 1.5 percent by weight of litharge and in the omission of Alpha-Chlor 33, was prepared as described in Example 1.

(c) A grease differing principally from that described in 6(a) in the incorporation of 1.5 percent of litharge. This grease also contained 2.6 percent of "Alpha-Chlor 33."

Comparison of the greases of Example 6 is provided in Table IV, wherein all values are expressed in percent by weight unless otherwise indicated.

Table IV

| Example No.                                                             | 6a    | 6b    | 6c    |
|-------------------------------------------------------------------------|-------|-------|-------|
| Mineral Oil <sup>1</sup>                                                | 58.23 | 59.25 | 57.14 |
| Naphthenic Bright Stock <sup>1</sup>                                    | 19.20 | 19.63 | 18.99 |
| Lime Flour                                                              | 4.87  | 4.53  | 4.68  |
| Acetic Acid                                                             | 4.16  | 4.16  | 4.16  |
| Caprylic Acid                                                           | 2.50  | 2.50  | 2.50  |
| Coconut Oil                                                             | 6.34  | 6.33  | 6.33  |
| Hydrogenated Tallow Fatty Acids                                         | 2.10  | 2.10  | 2.10  |
| Alpha-Chlor 33                                                          | 2.60  |       | 2.60  |
| Litharge                                                                |       | 1.50  | 1.50  |
| Timken OK Load, lbs.                                                    | 40    | 30    | 45    |
| Oxidation Stability, hrs. to 10 lbs. pressure drop, ASTM Bomb @ 210° F. | 75    | 62    | >200  |

<sup>1</sup> Same as in Example 1.

Data shown in Table IV reveal the surprising and unexpected results obtained by using lead and an extreme pressure additive together in the grease compositions of this invention.

As indicated by the illustrative examples shown herein, the greases of this invention have an excellent combination of desirable properties. The greases have long bearing life even under heavy and shock loads because of extreme pressure and anti-wear properties. They have outstanding resistance to rust and corrosion, and resist water wash-out in service. Because of their outstanding oxidation stability, they will lubricate for hundreds of hours at 300° F. and for thousands of hours at 250° F. Dropping points of greater than 500° F. indicate one reason for their remaining in place when subjected to high temperature operations. They are suitable for all types of lubricated surfaces, including anti-friction and plain bearings, cams, slides and the like. They are readily handled in dispensing and application equipment, as for centralized lubricating systems and pressure gun application.

The greases of this invention are suitable for a wide range of industrial application. Some, for example, are suitable for multi-purpose automotive greases, serving as chassis, wheelbearing, water-pump grease lubricant. Others are multi-purpose industrial greases serving as plain-bearing and anti-friction greases for normally loaded and heavily loaded equipment. In general, then, greases contemplated herein range from types suitable as textile machinery lubricants, to solid block type greases used in lubrication of machinery in steel mills, paper mills, cement mills, etc.

It is to be understood that the greases of this invention can also contain other characterizing materials and fillers. In particular, it has been found that certain antioxidants enhance the storage and shelf stability of the grease compositions. Outstanding among such materials is 2-6-ditertiary-butyl-4-methylphenol. Other such materials which may be used herein are: phenothiazine, diphenyl p-phenylene diamine, hexyl gallate, 4-tertiary butyl catechol, phenyl beta-naphthylamine, 2-4-ditertiary butyl p-cresol, tritertiary amyl phenyl phosphite together with a small amount of dicyclohexyl amine, polymerized trimethyl dihydroquinoline (Agerite resin of R. T. Vanderbilt Company), and mixtures of mono and diheptyl diphenylamines (Agerite Stalite of R. T. Vanderbilt Company).

I claim:

1. A grease composition, comprising: an oil of lubricating viscosity and a mixture (A) of alkaline earth metal soaps and salts therewith, the alkaline earth metals being selected from the group consisting of calcium and a mixture (B) of calcium and barium, not more than about fifteen percent of barium on a chemical equivalent basis being associated in said mixture (B) with calcium in said soaps and salts, the mixture (A) of said soaps and salts being present in a grease forming quantity, and the metal salts of said mixture (A) being salts of a low molecular weight unsubstituted saturated monocarboxylic acid (I) having from one to six carbon atoms per molecule, and

the metal soaps of said mixture (A) being soaps of different acids with said acid (I) as shown in the following tabulation:

| Acid                               | No. of Carbon Atoms | Weight Percent of Total Acids |
|------------------------------------|---------------------|-------------------------------|
| (I) Low Molecular Weight           | 1-6                 | 10-50                         |
| (II) Intermediate Molecular Weight | 7-12                | 5-50                          |
| (III) High Molecular Weight        | at least 13         | 5-40                          |
| (IV) Oil Acids                     | 8-18                | 25-60                         |

said acid (II) being selected from unsubstituted, mono-hydroxy-substituted and methyl-substituted saturated aliphatic monocarboxylic acids, said acids (III) being selected from unsubstituted and monohydroxy-substituted saturated aliphatic monocarboxylic acids and monounsaturated aliphatic monocarboxylic acids; and said oil acids being nut oil acids comprising mixtures of acids containing from about 8 to 18 carbon atoms per molecule and predominating in  $C_{12}$ - $C_{14}$  acids; from about 0.5 to about 5 percent by weight (expressed as PbO) of at least one lead compound of at least one of said acids (I) through (IV); and from about 1 to about 10 percent by weight of an extreme pressure agent containing at least one of the elements selected from the group consisting of chlorine, sulfur and phosphorus.

2. A grease as defined by claim 1 wherein the oil is a mineral oil.

3. A grease as defined by claim 1 wherein the alkaline earth metal is calcium.

4. A grease as defined by claim 1 wherein the low molecular weight acid (I) is acetic acid.

5. A grease as defined by claim 1 wherein the intermediate molecular weight acid (II) is caprylic acid.

6. A grease as defined by claim 1 wherein the high molecular weight acid (III) is stearic acid.

7. A grease as defined by claim 1 wherein the oil acids are coconut oil fatty acids.

8. A grease as defined by claim 1 wherein the oil acids are provided in the form of coconut oil.

9. A grease as defined by claim 1 wherein the extreme pressure agent is methyl dichlorostearate.

10. A grease as defined by claim 1 wherein the extreme pressure agent is a chlorinated sperm oil containing about thirty-three percent by weight of chlorine.

11. A grease composition comprising: (a) from about fifty to about ninety-eight percent by weight of an oil lubricating viscosity; (b) from about one to about forty percent by weight of a mixture of calcium salts and soaps of acids interrelated as shown below:

| Acid                               | No. of Carbon Atoms | Weight Percent of Total Acids |
|------------------------------------|---------------------|-------------------------------|
| (I) Low-Molecular Weight           | 1-6                 | 10-50                         |
| (II) Intermediate Molecular Weight | 7-12                | 5-50                          |
| (III) High Molecular Weight        | at least 13         | 5-40                          |
| (IV) Coconut Oil Acids             | 8-18                | 25-60                         |

(c) from about 0.5 to about 5 percent by weight (expressed as PbO) of a lead soap of at least one of said acids (I) through (IV); and (d) from about one to about ten percent by weight of an extreme pressure agent containing at least one of the elements selected from the group consisting of chlorine, sulfur and phosphorus.

12. A grease as defined by claim 11 wherein the coconut oil acids are provided in the form of coconut oil.

13. A grease as defined by claim 11 wherein the oil is a mineral oil.

5. 14. The method of preparing a grease composition, comprising: (a) charging to a reaction vessel in the order named and heating together at a temperature from about 250° F. to about 350° F.: an oil of lubricating viscosity; a calcium compound selected from the group consisting of an oxide, a hydroxide and a carbonate; a low molecular weight unsubstituted monocarboxylic acid (I) having from one to six carbon atoms per molecule; a minor quantity of water; an intermediate molecular weight monocarboxylic acid containing from seven to twelve carbon atoms per molecule and selected from the group consisting of an unsubstituted, a monohydroxy-substituted and a methyl-substituted saturated aliphatic acid; coconut oil acids; a high molecular weight aliphatic monocarboxylic acid containing at least thirteen carbon atoms per molecule and selected from the group consisting of an unsubstituted acid, a monohydroxy-substituted acid and a monounsaturated acid; and litharge; (b) dehydrating the mixture formed in (a), at a temperature from about 300° F. to about 350° F. at atmospheric pressure;

15. 16. incorporating into the resultant product of (b), at a temperature below about 300° F., an extreme pressure agent containing at least one of the elements selected from the group consisting of chlorine, sulfur and phosphorus; (d) the proportions of said materials being as defined in claim 3.

17. The method of preparing a grease composition, comprising: (a) charging to a reaction vessel in the order named and heating together at a temperature from about 250° F. to about 350° F.: a mineral oil, lime flour, acetic acid, a minor quantity of water, caprylic acid, coconut oil, stearic acid and litharge; (b) dehydrating the mixture formed in (a), at a temperature from about 300° F. to about 350° F. at atmospheric pressure; (c) incorporating into the resultant product of (b), at a temperature below about 300° F., an extreme pressure agent containing at least one of the elements selected from the group consisting of chlorine, sulfur and phosphorus; (d) the proportions of said materials being as defined in claim 3.

18. The method of claim 15 wherein step (a) is conducted at a pressure up to about 200 pounds per square inch.

19. The method of claim 15 wherein additional mineral oil is added to the resultant product of (b) before step (c).

20. 21. The method of claim 15 wherein the grease formed in (c) is homogenized.

22. The method of claim 15 wherein an antioxidant is added in step (c).

#### 55 References Cited in the file of this patent

#### UNITED STATES PATENTS

|           |                  |               |
|-----------|------------------|---------------|
| 2,229,042 | Brunstrum et al. | Jan. 21, 1941 |
| 2,319,405 | Ittner           | Mar. 18, 1943 |
| 2,457,586 | McGrogan         | Dec. 28, 1948 |
| 2,583,394 | Schott et al.    | Jan. 22, 1952 |
| 2,704,363 | Armstrong        | Mar. 15, 1955 |
| 2,846,392 | Morway et al.    | Aug. 5, 1958  |
| 2,863,847 | Morway           | Dec. 9, 1958  |

UNITED STATES PATENT OFFICE  
CERTIFICATE OF CORRECTION

Patent No. 2,898,297

August 4, 1959

John E. Schott

It is hereby certified that error appears in the printed specification of the above numbered patent requiring correction and that the said Letters Patent should read as corrected below.

Column 4, lines 67, 68, and 69, in the table, under the heading "Preferred Range" for

|        |      |         |
|--------|------|---------|
| 1-2    |      | 1-2     |
| 2-     | read | 2-5     |
| 0.2-0. |      | 0.2-0.6 |

column 8, line 34, for "Peneration" read -- Penetration --.

Signed and sealed this 9th day of February 1960.

(SEAL)

Attest:

KARL H. AXLINE

Attesting Officer

ROBERT C. WATSON  
Commissioner of Patents